

# UNITED STATES PATENT OFFICE.

PETER SCHMID, OF BASEL, SWITZERLAND.

## UNGUMMING RAW SILK.

No. 895,112.

Specification of Letters Patent.

Patented Aug. 4, 1908.

Application filed July 6, 1907. Serial No. 382,536.

*To all whom it may concern:*

Be it known that I, PETER SCHMID, a citizen of the Swiss Republic, and resident of Basel, Switzerland, have invented a new and 5 useful Improvement in the Ungumming of Raw Silk, of which the following is a full, clear, and exact specification.

The improvement in the ungumming of raw silk (such as silk, silk waste, spun silk, fabrics 10 of silk or silk waste), forming the subject of this invention, consists in conveying an electric current through the soap solution, in form of lather or of a liquid bath, with which the raw silk is to be treated, whereby the 15 duration of the treatment is materially shortened.

Example. Two electrodes of a material, which is not affected by the soap lather and which is a conductor of electricity, are ar- 20 ranged in a suitable apparatus for the treat- 25 ment of raw silk by means of soap lather in accordance with the process described in my United States Letters Patent No. 848,605 dated March 26th 1907, the walls of the ap- 30 paratus not being conductors of electricity, and the said electrodes being arranged at opposite sides of the apparatus, and in such a manner that they extend through the whole depth of the soap lather, but do not come into 35 contact with the silk to be treated. These electrodes are connected up in an electric circuit so that the density of the current which circulates between them is from  $\frac{1}{2}$  to 2 amperes and over per square decimeter of 40 electrode surface, while the tension of the current varies in accordance with the distance separating the said electrodes. For a distance of 44 centimeters the tension would be, for example, 120 volts. The electric current 45 which circulates through the soap lather and eventually also through the soap solution beneath the same considerably increases the action of the said lather so that the time requisite for softening or dissolving the gummy matter (sericin) is materially diminished. The result of this shortening of

the duration of the operation is that the silk fibers acquire a higher degree of elasticity, greater strength and increased gloss by reason of the reduced time during which it is 50 maintained in contact with the soap lather.

The time requisite for the ungumming of the raw silk is likewise reduced when the electric current is employed in the usual process for the treatment of the silk, wherein 55 the raw silk is subjected to the action of a soap solution in form of a liquid bath. In this case, two electrodes, which are unaffected by the soap bath, are arranged at opposite ends of a 60 vat of wood or other material which is not a conductor of electricity, in such a manner that they extend from the top to the bottom of the soap solution contained in the vat and are connected up in an electric circuit, in such a way that the current flowing through 65 the latter circulates through the soap solution during the treatment, the silk being treated in the usual way during this operation, that is to say, being moved in the bath. In either case, that is to say, whether the proc- 70 ess is carried out by means of a soap bath or by soap lather, the conductivity of the bath or of the lather may be increased by a small addition of sodium phosphate or sodium acetate. 75

What I claim is:

The described improvement in the ungum- 80 ming of raw silk consisting in passing an elec- 85 tric current through the soap solution with which the silk is treated while the said silk is in contact with the said soap solution for the purpose of reducing the duration of the opera- 90 tion and of obtaining a silk fiber which pos- 95 sses more gloss, strength and elasticity than hitherto. 85

In witness whereof I have hereunto signed my name this 22 day of June 1907, in the presence of two subscribing witnesses.

PETER SCHMID.

Witnesses:

GEO. GIFFORD,  
AMAND RITTER.